

## UNITED STATES PATENT OFFICE

2,320,228

## LUBRICANT

Delton R. Frey, East Cleveland, Ohio, assignor to  
The Lubri-Zol Corporation, Wickliffe, Ohio, a  
corporation of Ohio

No Drawing. Application July 18, 1940,  
Serial No. 346,219

14 Claims. (Cl. 252—38)

This invention relates as indicated to lubricating compositions and more particularly to lubricating compositions which are designed for use as crank case lubricants, and especially where high temperatures and conditions otherwise severe are encountered.

It has been recognized for quite some time that the properties of a lubricating composition for use in internal combustion engines, such as for example the Diesel type, may be improved by the addition thereto of minor amounts of certain types of metallo organic compounds since the same have a detergent effect in keeping down the deposit of sludge and the like which ordinarily builds up in places such as behind the piston rings and otherwise interferes with the proper operation of the engine.

It has also been recognized that aromatic compounds are generally preferred as addition agents and consequently many of the commercially successful addition agents for lubricants of this character have been of the aromatic type. The desirability of using an aryl metal oxide, i. e., an aromatic compound in which the oxygen of the metallic oxide group is directly attached to the aromatic nucleus, has also been recognized. Such compounds, unless further modified, however, are only very slightly, if at all, oil-soluble. It becomes necessary, therefore, to modify such aryl metal oxides in some way so that they may be dissolved in the mineral oil.

Reiff in U. S. Patent No. 2,197,833 modified these aryl metal oxides by replacing one or more of the nuclear hydrogens with a hydrocarbon side chain, i. e., Reiff suggested alkylation of these compounds for the purpose of rendering them oil-soluble.

The compounds proposed by Reiff are, however, somewhat difficult to manufacture, and are consequently quite expensive, and moreover do not possess certain properties which an addition agent of this character might desirably include.

It is a principal object of this invention, therefore, to provide a lubricating composition of the character described in which the addition agent is not only an improvement in its effectiveness over those available in the prior art, but which may be manufactured at a relatively low cost.

Other objects of this invention will appear as the description proceeds.

To the accomplishment of the foregoing and related ends, said invention then comprises the features hereinafter fully described and particularly pointed out in the claims, the following description setting forth in detail certain illustrative embodiments of the invention, these being indicative, however, of but a few of the various ways in which the principle of the invention may be employed.

Broadly stated, this invention comprises the

discovery that an improved lubricating composition may be prepared by the addition to a mineral lubricating oil base of minor amounts of oil-soluble metal oxides of aromatic esters which oxides are of the type in which the oxygen of the metal oxide group is directly attached to an aromatic ring.

While it is believed that the foregoing definition of the broad class of addition agents whose use is contemplated by the present invention is thus accurately defined, nevertheless, for a more specific identification of the particular compounds which are representatives of such class, reference may desirably be had to the mode of preparation of the same, since, in this way, the particular type of compound can perhaps be more accurately identified than in any other way. A specific example will first be given, and then an indication will be given of the similar materials which may be prepared in the same way.

Such specific example may be referred to as magnesium lauryl salicylate, although it is preferred to identify the same as the organic magnesium oxide obtained by replacing the hydroxyl hydrogen of lauryl salicylate with magnesium. This specific example may be prepared in the following manner:

The first step in the preparation of the material is to prepare the ester, i. e., lauryl salicylate. This method in general consists of refluxing a slight excess of lauryl alcohol with salicylic acid using xylene, for example, as a water carrier. The material was refluxed for about twenty hours, after which it was made neutral to phenolphthalein with dilute caustic, and washed free of soap with warm water. The excess alcohol and solvent were then removed by vacuum distillation. Final traces of alcohol, solvent and moisture are removed by heating to 250° C. under a vacuum of about 28". An oil bath was used as a heating medium. The following table gives precise values for the various factors of the reaction:

Table I

|    |                                                                        |         |
|----|------------------------------------------------------------------------|---------|
| 45 | Weight of alcohol recovered (gms) .....                                | None    |
|    | Moles alcohol recovered .....                                          | None    |
|    | Weight of acid recovered (in H <sub>2</sub> O sol.<br>as salt) .....   | 52 gms. |
| 50 | Moles acid recovered .....                                             | .4      |
|    | Weight of NaOH used in neutralization .....                            | 14 gms. |
|    | Cc. of aqueous caustic used .....                                      | 800     |
|    | Cc. of H <sub>2</sub> O used in washing (in 3 equal<br>portions) ..... | 2,400   |
| 55 | Time of reflux in hours .....                                          | 20      |
|    | Temp. of reflux, °C.:<br>Bath temperature .....                        | 175     |
|    | Vapor temperature .....                                                | 145     |

After the ester is thus prepared, the metallic derivative of the same may be prepared by react-

ing the ester in an alcohol solution with the necessary amount of metal. When the material identified for purposes of convenience as magnesium lauryl salicylate was prepared, the following procedure was employed:

One mole of magnesium was reacted with 2 moles of lauryl salicylate in a flask equipped with a reflux condenser and a mechanical stirrer. The flask was heated on a water bath. Two moles of the ester were dissolved in an equal volume of 99.95% methyl alcohol and magnesium turnings added. The reflux condenser was then attached and the water bath heated to 80° C.—the reaction mixture refluxed at about 70° C. The magnesium all dissolved after refluxing for 2½ hours. The refluxing was continued for 2½ hours after the solution of the magnesium was completed. The reflux condenser was then removed and the alcohol distilled off at atmospheric temperature. The residue was dissolved in twice its weight of benzene and filtered through paper to remove a slight cloud. The benzol was removed by distillation under a vacuum of about 28".

A typical batch sheet in the production of the material thus identified as magnesium lauryl salicylate is as follows:

Table II

|                               |         |
|-------------------------------|---------|
| Grams lauryl salicylate       | 220     |
| Moles lauryl salicylate       | .72     |
| Grams magnesium               | 8.7     |
| Moles magnesium               | .36     |
| Cc. of 99.95% methyl alcohol  | 250     |
| Cc. of benzol                 | 500     |
| Grams of product recovered    | 225     |
| Time of reaction              | 5 hours |
| Temperature of reaction, °C.: |         |
| Bath                          | 80      |
| Reflux                        | 70      |

In addition to the foregoing description of the mode of manufacture of the material identified as magnesium lauryl salicylate, it is believed that it may be helpful to give below the procedure followed in the preparation of two other similar metal oxides, i. e., materials which may, for convenience, be identified as calcium lauryl salicylate and magnesium iso-amyl salicylate. The following procedure was followed:

Two moles of lauryl salicylate in methyl alcohol solution are reacted with one mole of calcium. The reaction is conducted in a flask equipped with a reflux condenser and a mechanical stirrer. The laurel ester was dissolved in an equal volume of 99.95% methyl alcohol. To this solution was added the required amount of metallic calcium. The calcium was cut into small pieces before adding it to the solution. The reaction vessel was then placed in a water bath and heated until the reaction started. The temperature at which the reaction starts was 70° C. (the reflux temperature). The reaction is exothermic, therefore, the bath should be removed as soon as the reaction starts. If the reaction becomes too violent, the flask may be immersed in a water bath until the reaction subsides. In about one hour, all of the calcium was dissolved. At this point, the water bath was heated to 80° C. and this temperature maintained for an additional two hours. The reflux condenser was then removed and the methyl alcohol distilled off at atmospheric pressure. The residue was dissolved in twice its weight of benzol. The solution was then filtered through paper to remove the slightly cloudy appearance.

The filtrate was returned to the flask and the benzol distilled off at a pressure of 6 cm. of Hg. The water bath was heated to boiling and held there for 15 minutes to insure the complete removal of the benzol.

A typical batch sheet in the production of calcium lauryl salicylate is as follows:

Table III

|                                |         |
|--------------------------------|---------|
| 10 Grams lauryl salicylate     | 100     |
| Moles lauryl salicylate        | .33     |
| Grams calcium                  | 6.1     |
| Moles calcium                  | .15     |
| Cc. of 99.95% methyl alcohol   | 100     |
| Cc. of benzene                 | 200     |
| Grams product                  | 98      |
| Time of reaction               | 3 hours |
| Reflux temp. of solution about |         |
| Temperature of reaction        | 70° C.  |
| Bath temperature               | 80° C.  |

In the preparation of magnesium iso-amyl salicylate, the same general procedure as outlined above was followed. However, the reaction between the magnesium and the iso-amyl salicylate is more violent than the reaction between magnesium and lauryl salicylate, therefore, the procedure used is the same as that given for the preparation of calcium lauryl salicylate, except that more benzol is required to dissolve the product.

A typical batch sheet in the preparation of magnesium iso-amyl salicylate is given in the following table:

Table IV

|                              |                               |
|------------------------------|-------------------------------|
| Grams of iso-amyl salicylate | 208                           |
| Moles of iso-amyl salicylate | 1.00                          |
| Grams of magnesium           | 12                            |
| Moles of magnesium           | .50                           |
| Cc. of 99.95% methyl alcohol | 300                           |
| Cc. of benzene               | 400                           |
| Grams of product             | 215                           |
| Time of reaction             | 4 hours                       |
| Temperature of reaction      | Reflux temp. of the solution. |

It will be observed that the aromatic ester of the specific examples given above from which a metal oxide was then prepared was, in each instance, an ester of salicylic acid with lauryl alcohol. The present invention is not limited to this particular ester as the base for the oxide. Any aromatic ester containing a hydroxyl group attached to an aromatic ring may be used.

In the preparation of the aromatic hydroxy esters in which the hydroxyl group is attached to an aromatic ring, and which are then used in the preparation of the metal oxide addition agents of the present invention, ester forming constituents from classes I and II given below may be combined.

|                               |  |
|-------------------------------|--|
| I. Organic acids              |  |
| (A) Phenolic acids            |  |
| Monohydroxy benzoic acids     |  |
| Salicylic acid                |  |
| p-Hydroxybenzoic acid         |  |
| m-Hydroxybenzoic acid         |  |
| Polyhydroxy benzoic acids     |  |
| Dihydroxybenzoic acids        |  |
| Protocatechuic acid           |  |
| Gentisic acid                 |  |
| Resorcylic acids              |  |
| Gallic acid                   |  |
| Hydroxyphenyl fatty acids     |  |
| Hydroxyphenyl acetic acids    |  |
| Hydroxyphenyl propionic acids |  |
| o-Hydroxycinnamic acid        |  |
| o-Hydroxybenzoyl acetic acid  |  |
| Hydroxy phthalic acids        |  |
| Hydroxy naphthoic acids       |  |

|                                               |    |                                                     |
|-----------------------------------------------|----|-----------------------------------------------------|
| Alkylated hydroxybenzoic acids                | 5  | Ethyl phenols                                       |
| Hydroxy tolue acids                           |    | Propyl phenols                                      |
| Hydroxy xylie acids                           |    | Butyl phenols                                       |
| Trimethyl hydroxybenzoic acids                |    | Amyl phenols                                        |
| Amyl hydroxybenzoic acids                     |    | Octyl phenols                                       |
| Octyl hydroxybenzoic acids                    |    | Lauryl phenols                                      |
| Lauryl hydroxybenzoic acids                   |    | Cetyl phenols                                       |
| Cetyl hydroxybenzoic acids                    |    | Cyclohexyl phenols                                  |
| Cyclo-alkyl substituted hydroxybenzoic acids: |    | Aryl-substituted phenols                            |
| Cyclohexyl hydroxybenzoic acids               |    | phenyl phenols                                      |
| Aryl hydroxybenzoic acids                     | 10 | Naphthols                                           |
| Phenyl salicylic acids                        |    | Guaiacol                                            |
| Hydroxyphenyl benzoic acids                   |    | 2. Polyhydric phenols                               |
| Hydroxy diphenic acids                        |    | Dihydroxybenzenes                                   |
| (B) Other acids                               |    | Catechol                                            |
| 1. Aliphatic                                  |    | Resorcinol                                          |
| Fatty acids                                   |    | Hydroquinone                                        |
| Acetic acid                                   |    | Alkylated and cyclo-alkylated dihydroxy-            |
| Propionic acid                                |    | benzenes                                            |
| Lauric acid                                   | 15 | Orcinol                                             |
| Stearic acid                                  |    | Hexylresorcinol                                     |
| Oleic acid                                    |    | Trihydroxybenzenes                                  |
| Ricinoleic acid                               |    | Pyrogallol                                          |
| 2. Cyclo-aliphatic acids                      |    | Phloroglucinol                                      |
| Naphthenic acids                              |    | Hydroxyquinol                                       |
| 3. Aromatic                                   | 20 | Dihydroxy diphenyls                                 |
| Benzolic acid                                 |    | Diphenols                                           |
| Aryl benzoic acids                            |    | Phenyl dihydroxybenzenes                            |
| Phenyl benzoic acids                          |    | Dihydroxy naphthalenes                              |
| Alkyl benzoic acids                           |    | Naphtho-dihydroxybenzenes                           |
| Toluic acids                                  |    | Dinaphthols                                         |
| Xylie acids                                   |    | Dihydroxybenzophenones                              |
| Lauryl benzoic acids                          |    | Benzoyl catechols                                   |
| Cyclohexyl benzoic acids                      |    | Benzoyl resorcinols                                 |
| Phthalic acid                                 |    | Salicyl phenols                                     |
| Alkylated phthalic acids                      |    | Esters of dihydroxybenzoic acid                     |
| Butyl phthalic acids                          |    |                                                     |
| Amyl phthalic acids                           |    |                                                     |
| Octyl phthalic acids                          |    |                                                     |
| Lauryl phthalic acids                         |    |                                                     |
| Diphenic acid                                 | 25 | It will be observed, that in order for the ester    |
| Naphthoic acids                               |    | to contain a hydroxyl group attached to an aro-     |
| Aryl fatty acids                              |    | matic ring, the ester must be formed from either    |
| Phenyl acetic acid                            |    | a phenolic acid and any alcohol, or from a phe-     |
| Phenyl propionic acid                         |    | nolic alcohol and any acid. Thus such aromatic      |
| Benzoyl benzoic acid                          | 30 | hydroxy esters may be prepared by combining         |
| II. Alcohols and phenols                      |    | any one of the phenolic acids of class IA above     |
| (A) Phenolic alcohols                         |    | with any of the esterifying materials of class      |
| Monohydroxy benzyl alcohols                   |    | II above, or alternatively by combining any of      |
| Saligenin (salicyl alcohol)                   |    | the phenolic alcohols of class IIA above with any   |
| p-Hydroxybenzyl alcohol                       |    | of the organic acids of class I above.              |
| m-Hydroxybenzyl alcohol                       | 35 | One type of hydroxy aromatic ester from             |
| Polyhydroxy benzyl alcohols                   |    | which the addition agents of this invention may     |
| Dihydroxy benzoic alcohols                    |    | be prepared by replacing the hydroxyl hydrogen      |
| Hydroxyphenyl-ethyl alcohols                  |    | with a metal, are those esters which may be made    |
| o-Hydroxyphenyl-ethyl alcohol                 | 40 | from polyhydroxyl phenols by esterifying only       |
| Hydroxyphenyl-cyclohexanols                   |    | part of the hydroxyl groups so that the final ester |
| Hydroxyphenyl-sterols                         |    | has at least one unesterified hydroxyl group at-    |
| Hydroxyphenyl-octyl alcohols                  |    | tached to an aromatic ring. A list of polyhydric    |
| Hydroxyphenyl-lauryl alcohols                 | 45 | phenols from which esters of this type may be       |
| Hydroxyphenyl-cetyl alcohols                  |    | prepared is given above under II CZ. For exam-      |
| Hydroxybenzyl alcohols                        |    | ple, a mono ester of resorcinol may be prepared     |
| Hydroxybenzyl benzyl alcohols                 |    | by esterifying one of the hydroxyl groups with      |
| Hydroxybenzyl ethyl alcohol                   | 50 | an acid such as naphthenic, stearic, phenyl-        |
| Hydroxybenzyl lauryl alcohol                  |    | stearic, and chlorphenylstearic acids, and the hy-  |
| Coniferyl alcohol                             |    | drogen of the remaining phenolic hydroxy group      |
| (B) Other alcohols                            |    | replaced with a metal to form one type of the       |
| 1. Aliphatic                                  |    | addition agents of this invention.                  |
| Methyl alcohol                                | 55 | The thio esters will also be found to be of par-    |
| Ethyl alcohol                                 |    | ticular utility as the base for the metal oxide ad- |
| Propyl alcohols                               |    | dition agent of the present invention. Such thio    |
| Butyl alcohols                                |    | esters may for example be conveniently prepared     |
| Amyl alcohols                                 |    | in the well-known manner by reacting a phenolic     |
| Octyl alcohols                                |    | aromatic acid with a thio alcohol (for example      |
| Lauryl alcohols                               | 60 | benzyl mercaptan).                                  |
| Cetyl alcohols                                |    | In addition to calcium and magnesium, other         |
| Cyclo-aliphatic alcohols                      |    | metals of the alkaline earth group may be used      |
| Cyclohexanol                                  |    | to replace the hydroxyl hydrogen of the phenolic    |
| Methyl cyclohexanol                           |    | esters employed in the preparation of the metal     |
| Amyl cyclohexanol                             |    | oxide, the use of which in lubricants is contem-    |
| Cyclohexyl cyclohexanol                       |    | plated in the present invention. In addition,       |
| Menthol                                       | 65 | metals of other groups, for example aluminum,       |
| Terpineol                                     |    | zinc, cobalt and nickel, may also be employed,      |
| Sterols                                       |    | but in this case a method of preparation differ-    |
| Naphthyl alcohols                             | 70 | ent from that used in the above examples is usu-    |
| 2. Aromatic                                   |    | ally required. This may consist of replacing the    |
| Benzyl alcohol                                |    | hydroxyl hydrogen with an alkali metal and then     |
| Alkylated and cyclo-alkylated benzyl alcohols |    | reacting the phenate thus formed with an alco-      |
| Methyl benzyl alcohols                        |    | hol-soluble salt with the desired metal in alco-    |
| Ethyl benzyl alcohols                         |    | holic solution. Alternatively the sodium deriva-    |
| Propyl benzyl alcohols                        |    |                                                     |
| Amyl benzyl alcohols                          |    |                                                     |
| Lauryl benzyl alcohols                        |    |                                                     |
| Cetyl benzyl alcohols                         |    |                                                     |
| Cyclohexyl benzyl alcohols                    |    |                                                     |
| Arylated benzyl alcohols                      |    |                                                     |
| Phenyl benzyl alcohols                        |    |                                                     |
| Benzhydrol                                    |    |                                                     |
| Triphenylcarbinol                             |    |                                                     |
| Xenyl benzyl alcohols                         |    |                                                     |
| Naphthyl benzyl alcohols                      |    |                                                     |
| Phenyl ethyl alcohols                         |    |                                                     |
| Phenyl propyl alcohols                        |    |                                                     |
| Benzoin                                       |    |                                                     |
| (C) Phenols                                   |    |                                                     |
| 1. Monohydric phenols                         |    |                                                     |
| Phenol                                        |    |                                                     |
| Alkylated and cyclo-alkylated phenols         |    |                                                     |
| Cresols                                       |    |                                                     |
| Xylenols                                      |    |                                                     |
| Carvacrol                                     |    |                                                     |
| Thymol                                        |    |                                                     |

tive of the hydroxy ester may be formed and the latter reacted with an alcohol-soluble salt of the desired metal in alcoholic solution.

In addition to the metal oxide and ester groups which characterizes the addition agents of this invention, other substituents may also advantageously be present in the compound, attached either to an aromatic ring or at some other point. These may be any of the following:

## IV. The halogens

Fluorine  
Chlorine  
Bromine  
Iodine

## II'. Oxygen-bearing radicles

These may be classified according to the nature of the attachment of the oxygen to the molecule, viz:

(A') Directly attached to one or more carbon atoms as in the case of:

(1') The ether radicle,  $-\text{O}-$

(2') The hydroxyl radicle,  $-\text{OH}$

(3') The carbonyl radicle,  $-\text{C=O}$

And other radicles containing Carbonyl, e. g.



(4') Radicles in which oxygen forms part of a ring structure, e. g.

Furyl and hydrofuryl

(5') Inorganic radicles where the Oxygen is directly attached to a Carbon atom, e. g.

Arsenite

Hypochlorite

Phosphate

Thiophosphate

Thiophosphite

$\beta$ -Hydroxylamine

Borate

(B') Indirectly attached through the means of some other atom, as in the form of an inorganic radicle, e. g.

Arsenate

Chlorate

Chlorite

Cyanate

$\alpha$ -Hydroxylamine

Nitrate

Nitrite

Nitro

Nitroso

Oxime

Perchlorate

Phosphate

Sulphate

Sulphite

Sulphinic acid

Sulphone

Sulphonic acid

Sulphoxide

Thiophosphate

Thiophosphite

Thio-sulphate

(Note: This class includes salts of organic bases with inorganic oxy-acids.)

## III'. Other substituent groups including:

Amino, and substituted amino  
Imino  
Azo  
Hydrazo  
Hydrazine  
Nitrile  
Isonitrile  
Mercapto  
Sulphide  
Polysulphide  
Thiocyanate  
Thiocarbonyl  
Thio-amide  
Dithio-amide  
Dithio-carboxyl (including ester and salt groups derived therefrom)

It will be noted that the substituent groups referred to above include those which contain elements other than carbon, hydrogen, and oxygen.

15 The term "inorganic substituents" is used in the appended claims in defining these. Examples of such inorganic substituents given above are those which consist of or which contain the halogens, sulphur, nitrogen, phosphorus, arsenic, boron, and the metals.

20 The base oil in which the addition agents of the present invention may be advantageously employed may be any lubricating oil commonly used for the purposes previously defined. It is one advantage of these addition agents that they are effective in both naphthenic and paraffinic base oils.

25 The addition agents of the present invention will generally be found to give best results if employed in concentrations of from 0.05% to 10% and usually from 0.1% to 5% in highly refined mineral lubricating oils. A concentration of about 1.5% will usually be found to give best results when used in a highly refined paraffinic or naphthenic base oil, and used for the purpose of lubricating a Diesel engine. It is conceivable that among the various materials specifically identified above from which the metal oxide addition agents of the present invention may be prepared, certain metal oxides may be prepared which are not sufficiently oil-soluble. They, of course, are not intended to be included in the definition of the addition agents in the appended claims, where, it will be observed, the limitation oil-soluble is used.

30 Where an exceptionally high film strength oil is desired, i. e., a finished lubricant which has improved detergent as well as film strength properties, the addition agents of the present invention may be employed in conjunction with a separate extreme pressure addition agent such as a sulphur or halogen compound, and optionally a halogen such as chlorine may be included 35 in the addition agents themselves, so that both high detergency and high film strength may be the property possessed by the same molecule.

35 Throughout the foregoing description of the addition agents, the use of which in lubricants is contemplated by this invention, they have been generally referred to as metal oxides of aromatic esters with the oxygen of the metal oxide group directly attached to an aromatic ring. The class 40 of materials which may be thus described, and of which representative examples have been given, have been prepared in such a way that it is logical to assume that in the reaction between the metal and the ester, the metal, during the ensuing reaction, replaces the hydroxyl hydrogen. 45 No reason is apparent why the reaction does not take place as thus assumed. It is to be understood, however, that irrespective of the precise reaction which takes place in the preparation of the materials as above identified, the present invention contemplates the use of end products of

the character of those which may be prepared by one of the methods described herein, irrespective of whether the reaction between the metal and the ester in the formation of the addition agent is precisely that which has been assumed. For convenience in designation, however, the terminology above given, i. e., organic metal oxide of aromatic esters in which the oxygen of the metal oxide group is attached to an aromatic ring, is employed in the appended claims for the purpose of designating the type of materials which have been found satisfactory, and to which this invention thus relates.

Representative examples of lubricating compositions of the present invention were tested by means of a 2½ H. P. single-cylinder, liquid-cooled, four cycle gasoline engine, rated at 1800 R. P. M. The procedure used was as follows:

The engine was loaded by means of a fan-type brake which applied a load of 1½ H. P. at 1600 R. P. M. The engine was run for ten minutes at 1200 R. P. M. and then the speed was increased to 1600 R. P. M. The following conditions were maintained constant during the remainder of the test:

|                          |         |        |
|--------------------------|---------|--------|
| Coolant temperature..... | °F..... | 345    |
| Oil temperature.....     | °F..... | 225    |
| Air fuel ratio.....      |         | 12.7:1 |

The engine was stopped at 30 hour periods for inspection of piston, piston skirt, piston rings, connecting rod bearings, etc. The engine was equipped with removable connecting-rod bearings consisting of lead-bronze with a steel backing. These bearings were weighed at the beginning of the test and at each 30 hour inspection period. Before each new test, the engine was thoroughly cleaned and equipped with new piston, piston rings and with new connecting rod bearings.

In the following table will be found a tabulation of the characteristics of the lubricant tested, its comparison with an untreated base oil both as to physical properties and performance in the engine tests.

Other modes of applying the principle of my invention may be employed instead of the one explained, change being made as regards the composition and method herein disclosed, provided the ingredients or steps stated by any of the following claims or the equivalent of such stated ingredients or steps be employed.

I therefore particularly point out and distinctly claim as my invention:

- 10 1. A lubricating composition comprising a major proportion of mineral lubricating oil and a minor proportion of an oil-soluble metal oxide of an ester of an aromatic acid with an aliphatic alcohol, which oxide is of the type in which the oxygen of the metal oxide group is directly attached to an aromatic ring.
- 15 2. A lubricating composition comprising a major proportion of mineral lubricating oil and a minor proportion of an oil-soluble metal oxide of an ester of an aromatic acid with a long chain aliphatic alcohol, which oxide is of the type in which the oxygen of the metal oxide group is directly attached to an aromatic ring.
- 20 3. A lubricating composition comprising a major proportion of mineral lubricating oil and a minor proportion of an oil-soluble metal oxide of an ester of salicylic acid, which oxide is of the type in which the oxygen of the metal oxide group is directly attached to an aromatic ring.
- 25 4. A lubricating composition comprising a major proportion of mineral lubricating oil and a minor proportion of an oil-soluble metal oxide of an ester of salicylic acid and an aliphatic alcohol, which oxide is of the type in which the oxygen of the metal oxide group is directly attached to an aromatic ring.
- 30 5. A lubricating composition comprising a major proportion of mineral lubricating oil and a minor proportion of an oil-soluble metal oxide of an ester of salicylic acid and lauryl alcohol which oxide is of the type in which the oxygen of the metal oxide group is directly attached to an aromatic ring.
- 35 6. A lubricating composition comprising a major proportion of mineral lubricating oil and a minor proportion of an oil-soluble metal oxide of an ester of salicylic acid and an aliphatic alcohol, which oxide is of the type in which the oxygen of the metal oxide group is directly attached to an aromatic ring.
- 40 7. A lubricating composition comprising a major proportion of mineral lubricating oil and a minor proportion of an oil-soluble metal oxide of an ester of salicylic acid and lauryl alcohol which oxide is of the type in which the oxygen of the metal oxide group is directly attached to an aromatic ring.
- 45 8. A lubricating composition comprising a major proportion of mineral lubricating oil and

|                                        | Example No. I |                                     | Example No. II |                                     |
|----------------------------------------|---------------|-------------------------------------|----------------|-------------------------------------|
|                                        | Naphthenic    | Naphthenic Mg.<br>Lauryl salicylate | Paraffinic     | Paraffinic Mg.<br>Lauryl salicylate |
| Type of oil.....                       | Naphthenic    | Naphthenic Mg.<br>Lauryl salicylate | Paraffinic     | Paraffinic Mg.<br>Lauryl salicylate |
| Addition agent.....                    | None          | 1.00                                | 1.00           | 1.00                                |
| Percent added.....                     |               | .065                                |                | .063                                |
| Per cent ash.....                      | 0             | 0                                   | 0              | 0                                   |
| Acid number.....                       | 0.03          | Basic 0.04                          | 0.04           | Basic 0.03                          |
| Conradson carbon.....per cent.....     | 0.06          | 0.22                                | 0.67           | 0.85                                |
| Viscosity at 210° F.....               | 55.2          | 56.5                                | 58.0           | 59.0                                |
| Viscosity at 100° F.....               | 60.1          |                                     | 38.1           |                                     |
| A. P. I. gravity.....                  | 19.7          |                                     | 29.9           |                                     |
| Flash point.....°F.....                | 390           |                                     | 445            |                                     |
| Fire point.....°F.....                 | 430           |                                     | 490            |                                     |
| Pour point.....°F.....                 | -5            |                                     | 10             |                                     |
| N. P. A. color.....                    | 2             |                                     | 6              |                                     |
| Engine test, piston condition at—      |               |                                     |                |                                     |
| 60 hrs.....                            | D             | A+                                  | D              | A+                                  |
| 90 hrs.....                            |               | A                                   |                | A+                                  |
| 120 hrs.....                           |               | A                                   |                | A                                   |
| 150 hrs.....                           |               | A-                                  |                | A                                   |
| 180 hrs.....                           |               | (1)                                 |                | A                                   |
| Number of rings stuck at—              | 1             | None                                | 2              | None                                |
| 60 hrs.....                            |               | do                                  |                | do                                  |
| 90 hrs.....                            |               | do                                  |                | do                                  |
| 120 hrs.....                           |               | do                                  |                | do                                  |
| 150 hrs.....                           |               | do                                  |                | do                                  |
| 180 hrs.....                           |               | (1)                                 |                | do                                  |
| Per cent filling of oil ring slots at— | 90            | 0                                   | 85             | 0                                   |
| 60 hrs.....                            |               | 0                                   |                | 0                                   |
| 90 hrs.....                            |               | 0                                   |                | 0                                   |
| 120 hrs.....                           |               | 0                                   |                | 0                                   |
| 150 hrs.....                           |               | 0                                   |                | 0                                   |
| 180 hrs.....                           |               | (1)                                 |                | 0                                   |
| Loss in weight of bearings, mgs. at—   |               |                                     |                |                                     |
| 60 hrs.....                            | 22            | 10.5                                | 8.4            | 19.5                                |
| 90 hrs.....                            |               | 16.5                                |                | 29.0                                |
| 120 hrs.....                           |               | 20.0                                |                | 38.5                                |
| 150 hrs.....                           |               | 24.5                                |                | 43.0                                |
| 180 hrs.....                           |               | (1)                                 |                | 65.0                                |

a minor proportion of an oil-soluble alkaline-earth metal oxide of an ester of salicylic acid and lauryl alcohol, which oxide is of the type in which the oxygen of the metal oxide group is directly attached to an aromatic ring.

7. A lubricating composition comprising a major proportion of mineral lubricating oil and a minor proportion of an oil-soluble organic magnesium compound of the type which may be produced by reacting metallic magnesium with an ester of salicylic acid in the presence of an alcohol.

8. A lubricating composition comprising a major proportion of mineral lubricating oil and a minor proportion of the organic magnesium oxide obtained by replacing the hydroxyl hydrogen of lauryl salicylate with magnesium.

9. A lubricating composition comprising a major proportion of mineral oil and a minor proportion of an oil-soluble metal oxide of an aromatic ester in which the metal oxide group is directly attached to an aromatic ring, having the general formula



where M is a metal, R is an aromatic radical, X is selected from the class consisting of sulphur and oxygen, X' is selected from the class consisting of oxygen and sulphur, and R' is selected from the class consisting of aromatic radicals, cycloaliphatic radicals, and aliphatic radicals.

10. A lubricating composition comprising a major proportion of mineral oil and a minor proportion of an oil-soluble metal oxide of an aromatic ester in which the metal oxide group is directly attached to an aromatic ring, having the general formula



where M is a metal, R is an aromatic radical, X is selected from the class consisting of oxygen and sulphur, X' is selected from the class consisting of oxygen and sulphur, and R' is selected from the class consisting of aromatic radicals, cycloaliphatic radicals, and aliphatic radicals, which organic metal oxide also contains an additional inorganic substituent in at least one of the radicals of the class consisting of R and R' in the foregoing formula.

11. A lubricating composition comprising a major proportion of mineral oil and a minor proportion of an oil-soluble metal oxide of an aromatic ester in which the metal oxide group is directly attached to an aromatic ring, having the general formula



where M is a metal, R is an aromatic radical, X is selected from the class consisting of oxygen and sulphur, X' is selected from the class consisting

of oxygen and sulphur, and R' is selected from the class consisting of aromatic radicals, cycloaliphatic radicals, and aliphatic radicals, which organic metal oxide also contains an inorganic substituent selected from the class consisting of sulphide and polysulphide radicals in at least one of the radicals of the class consisting of R and R' in the foregoing formula.

12. A lubricating composition comprising a major proportion of mineral oil and a minor proportion of an oil-soluble metal oxide of an aromatic ester in which the metal oxide group is directly attached to an aromatic ring, having the general formula



where M is a metal, R is an aromatic radical, X is selected from the class consisting of oxygen and sulphur, X' is selected from the class consisting of oxygen and sulphur, and R' is selected from the class consisting of aromatic radicals, cycloaliphatic radicals, and aliphatic radicals, which organic metal oxide also contains sulphur in at least one of the radicals of the class consisting of R and R' in the foregoing formula.

13. A lubricating composition comprising a major proportion of mineral oil and a minor proportion of an oil-soluble metal oxide of an aromatic ester in which the metal oxide group is directly attached to an aromatic ring, having the general formula



where M is a metal, R is an aromatic radical, X is selected from the class consisting of oxygen and sulphur, X' is selected from the class consisting of oxygen and sulphur, and R' is selected from the class consisting of aromatic radicals, cycloaliphatic radicals, and aliphatic radicals, which organic metal oxide also contains a halogen in at least one of the radicals of the class consisting of R and R' in the foregoing formula.

14. A lubricating composition comprising a major proportion of mineral oil and a minor proportion of an oil-soluble metal oxide of an aromatic ester in which the metal oxide group is directly attached to an aromatic ring, having the general formula



where M is a metal, R is an aromatic radical, X is selected from the class consisting of oxygen and sulphur, X' is selected from the class consisting of oxygen and sulphur, and R' is selected from the class consisting of aromatic radicals, cycloaliphatic radicals, and aliphatic radicals, which organic metal oxide also contains chlorine, in at least one of the radicals of the class consisting of R and R' in the foregoing formula.

DELTON R. FREY.